

June 30, 1942.

C. WESSEL

2,287,848

METHOD OF CASTING

Filed Jan. 16, 1939

3 Sheets-Sheet 1



Attorney  
Carl Wessel  
By  
Williams, Bradbury  
McCaleb & Hinckle  
Attnys

June 30, 1942.

C. WESSEL

2,287,848

METHOD OF CASTING

Filed Jan. 16, 1939

3 Sheets-Sheet 2



June 30, 1942.

C. WESSEL

2,287,848

METHOD OF CASTING

Filed Jan. 16, 1939

3 Sheets-Sheet 3



Inventor:  
Carl Wessel  
By  
Williams, Bradbury,  
McCalet & Hinckle  
Attest

## UNITED STATES PATENT OFFICE

2,287,848

## METHOD OF CASTING

Carl Wessel, Chicago, Ill., assignor, by mesne assignments, to Carl Wessel and Lew W. Cleminson, both of Chicago, Ill., trustees

Application January 16, 1939, Serial No. 251,092

9 Claims. (Cl. 22—57)

The present invention relates to methods of casting, and is particularly concerned with methods for producing better castings and better metal stock of various shapes more efficiently and more economically than can be done by the methods and apparatus of the prior art.

One of the objects of the present invention is the provision of an improved method of casting metal, utilizing refractory or metal molds, and filling the mold by gravity of the liquid metal in such manner that the complete filling of the mold is effected and the shrinkage is avoided by the continuous application of liquid metal under pressure, due to gravity head, while the casting is cooling from its most remote end toward the filling gate.

Another object of the invention is the provision of an improved method of casting by means of which extremely thin sections may be made and by means of which the freezing of a part of the metal during the pouring process, commonly referred to as blow-holes, may be eliminated.

Another object of the invention is the provision of an improved method of casting which produces an absolutely solid casting and produces a high degree of uniformity of crystal structure of the casting, and which is also economical in its operation.

Another object of the invention is the provision of an improved method of casting which avoids the contamination of the metal by filling the mold without the liquid metal coming in contact with any air except that small amount which is present in the mold.

Another object of the invention is the provision of an improved method of casting which is adapted to avoid shrinkage by means of the continuous application of metal in liquid form under pressure head due to gravity for a predetermined time, so that the congealation of the metal may be accomplished while pressure is applied.

Another object of the invention is the provision of improved methods which are not only adaptable for individual casting and small plants but for mass production.

Another object of the invention is the provision of an improved method of producing sheets, strips, and stock shapes of metal, by means of which much costly rolling and annealing equipment may be eliminated, and by means of which stock shapes thin enough and possessing the necessary homogeneity for finishing and rolling purposes may be made, thereby reducing the cost of production and capital required for equipment.

Another object of the invention is the provi-

sion of improved castings and methods for producing castings, by means of which shrinkage, flaws, and the formation of pipes and shrinking strains are eliminated, and castings of uniform crystal structure may be produced at a minimum cost.

Another object of the invention is the provision of an improved casting method which permits the melting and casting of the metal under reduced air, or controlled air conditions as required by the metal used.

Other objects and advantages of the invention will be apparent from the following description and the accompanying drawings, in which similar characters of reference indicate similar parts throughout the several views.

Referring to the three sheets of drawings which accompany this specification,

Fig. 1 is a diagrammatic top plan view of a plurality of melting furnaces arranged for discharge into a centrally located ladle;

Fig. 2 is a similar view of a modified furnace and ladle arrangement;

Fig. 3 is a horizontal sectional view, taken on the plane of the line 3—3 of Fig. 4, showing the structure of the ladle of Figs. 1 and 2;

Fig. 4 is a vertical sectional view, taken on the plane of the line 4—4 of Fig. 3, looking in the direction of the arrows, showing the structure of the ladle and the closely associated part of the mold;

Fig. 5 is a fragmentary sectional view of a modified form of connection between the ladle and the mold, which may be utilized in Fig. 4;

Fig. 6 is a fragmentary elevational front view of the front part of the ladle and conveying mechanism for supporting the molds in pouring position.

Referring to Figs. 1 and 2, these are diagrammatic arrangements of a plurality of furnaces, shown in connection with a ladle of the type illustrated in Figs. 3 and 4.

According to my method of operation in a foundry of suitable size, the ladle 20 is provided with an insulating lining 21 and is adapted to receive within its chamber 71 a suitable supply of molten metal for continuous casting operation.

The ladle 20 is a fixed ladle, and by means of its insulating lining 21 it maintains the metal at a suitable high degree of temperature for casting operations, the metal being discharged from the discharge aperture 23 at the lower part of the ladle 20.

The furnaces 23—26 may be arranged in a circle about the upper part of the ladle 20, that

is, on an upper floor, in such manner that each furnace may have its discharge conduit 27 of equal length to those of the other furnaces, and the furnaces are to be periodically charged with a batch of metal to be melted and successively discharged into the ladle 20.

Different numbers of melting furnaces may, of course, be employed, the furnaces preferably being of the rotating tilting type. For example, if four furnaces are employed, a batch might be discharged into the ladle every fifteen minutes, the capacity of each furnace being about 250 pounds per hour; while, if three furnaces were employed, a batch would be discharged every twenty minutes. Under these conditions the capacity of the ladle might be approximately 1200 pounds or two cubic feet, and the inner measurements of the ladle might be, for example, ten inches inner diameter by thirty inches high.

The temperature of the metal discharged from the furnaces might be approximately 2200 degrees F., and the temperature of the metal in the ladle might be slightly lower, but need not vary more than about 200 degrees F., as the heat of the metal in the ladle would be continuously replenished by the periodic discharge into the ladle of hotter metal from the furnaces.

Each furnace is preferably provided with a rotating discharge spout 21, and the ladle or reservoir 20 is preferably provided with a suitable cover, which is removable, so that the metal is enclosed from the time it is melted in the furnace and during its discharge into the ladle and during its discharge from the ladle into the mold, as will further be described.

A cleaning of the metal is effected in the furnace before the pouring operation by scraping out the dross and slag, with the furnace almost in level position, the scraping being effected through a discharge opening.

The melting may then be accomplished under reduced air and controlled conditions.

In the example of a furnace and ladle proportions cited, the head of pressure might vary from full head in the ladle to half head during most of the day's casting. At the end of the day's run, the reduced head, from one-half to zero in the ladle, would be utilized for the casting of relatively small molds, which would not require as much gravity head as the larger castings. The total capacity per day for an eight hour day of casting would be approximately 7,000 pounds.

As the practice of the method may be made more clear by reference to one example of the apparatus, I shall now describe in full one form of apparatus which may be used for practicing the invention.

Referring to Fig. 1, each of the melting furnaces 23-26 is, of course, provided with a suitable heating device, such as a gas or oil burner, and may be provided with a motor for rotating and each furnace of course comprises an internal firebrick insulation supported by a metal jacket as shown.

In Fig. 1 the discharge spouts, which are also provided with a metal jacket and a firebrick lining or refractory lining, may all be of the same length, thereby assuring equal temperature for the discharged metal from each of the furnaces.

In Fig. 2 the furnaces 30-33 each discharge 70 into the discharge conduits 34-37, and the two conduits 34, 35 and 36, 37 are jointly connected to conduits 38, 39 respectively. In this case the lengths of the conduits for all of the furnaces are not equal, but by means of the use of a suitable refractory 75

lining for the metal jacketed conduits 34-39 the excessive loss of heat can be practically eliminated and practically the same discharge temperature secured for the batch from each furnace.

In the event the end furnaces 30 and 33 give evidence of slightly greater cooling of the batch as it discharges down the elongated conduits 34, 38 and 37, 39, the end furnaces can be operated 10 at slightly higher temperatures, to effect equalization of the temperature of the batches discharged into ladle 20, which is similar in construction to the ladle or reservoir 20, previously described.

Referring to Figs. 3-6, these are detailed illustrations of the structure of the reservoir or ladle for melted metal and the arrangements for filling molds from this reservoir.

In Figs. 3 and 4 the ladle, which is indicated 20 in its entirety by the numeral 20, may have its interior insulation 21 formed in a plurality of layers, the layers comprising, respectively, the inner refractory 40, the firebrick 41, and the rock wool or asbestos fiber insulation 42.

The ladle 20 is preferably supported upon a suitable concrete foundation 43 and may have its external metal jacket 44 built up of a multiplicity of metal sections 45-51. These metal sections are in the form of endless metal bands of cylindrical shape, each successive section being supported upon the one below it so that the ladle 25 can be built to any desired height.

The metal jacket sections 45-51 are given additional support and held in alignment with each 35 other by a plurality of vertically extending eye beams 52-55 (Fig. 3), which are preferably equally spaced about the periphery of the metal jacket 44, extend axially thereof, and are located in contact with the external cylindrical surface 40 of the jacket sections 45-51.

At each joint between the jacket sections there is a metal band 56-61, and each metal band may be of similar construction to those shown in Fig. 45 3. The metal bands 56-61 are bent to substantially partially cylindrical form, and are long enough to encompass that portion of the periphery which is located between the flanges of a pair of eye beams 52-55. Any number of eye beams may be employed, but in a furnace of the size mentioned above I consider four eye beams sufficient, and the metal bands 61, for example, contact the external surfaces of the sections 50 and 51 of the jacket 44 throughout the major portion of their length, and are bent outward at 55 62 or provided with an offset 62 at each end so as to engage outside the inner flange 63 of the eye beams.

The band 61 is also provided with an attachment flange 64 extending radially at each end and adapted to engage the web 65 of the eye beam 54 or 55, and the attachment flanges 64 are provided with apertures for receiving the screw bolts 66, which pass through the attachment flanges 64 and through the web 65, and secure two of the attachment flanges of the bands 56-61 to each web.

The bands 56-61 are slightly shorter in length than the spaces between the webs of the respective eye beams 54, 55 so that there is a tolerance to be taken up by means of the bolts 66, which draw the bands tightly about the metal sections 45-51 the jacket 44 and assure the securement of these bands against vertical movement due to the frictional engagement between the bands and the metal sections.

The ladle also comprises an inner metal shell 70 of similar construction to the metal shell 44, or the inner metal shell may comprise the simple annular bands of metal, such as steel, mounted one upon the other in such a way as to overlap the joints between the firebricks. The space between the two shells 44 and 70 may be filled with rock wool, high temperature asbestos fiber, such as Amosite, glass wool, or quartz wool, for the purpose of conserving the heat in the ladle.

Inside the shell 70, the ladle 20 is provided with the layer 41 of firebrick, molded to fit together to form a wall which is annular in plan, and the firebrick preferably have their joints overlapping the joints between the sections of the inner shell 70. For example, if the firebrick are also one foot high, then this also facilitates the building of various sizes of ladles or reservoirs which differ in height by a foot.

The innermost layer of insulation comprises the refractory lining 40, which consists of a refractory composition that is smooth but not glazed, and which may be treated with flux or charcoal to prevent the metal from sticking to it.

The composition may include metal dioxides, clay, and feldspar, and such refractory linings may be made absolutely smooth so that the metal in the reservoir can be kept clean.

A de-oxidizer compound can be kept on top of the charge in the reservoir or ladle 20 for the purpose of preventing any air contamination.

The refractory lining 40 is also in the form of peripheral sections, which, for example, may be a foot high, and all of which fit together smoothly to form the cylindrical reservoir chamber 71 for receiving the molten metal. This chamber is substantially cylindrical in shape at its uppermost portion, such as, for example, the sections 72, 73, 74, or 75 but at its bottom the chamber 71 tapers in diameter and is curved laterally toward the discharge port 23. Thus the section 76 of the ladle chamber 71 tapers from the initial diameter to approximately half the diameter, and extends toward the left in Fig. 3, in a streamlined curve. The refractory blocks 77 adjacent this section are, of course, suitably formed for this purpose.

The refractory blocks 78 of the lowermost section have formed in them, when assembled, a continuation 79 of the tapered throat 76, which tapers still farther along smoothly curved lines toward the reduced conduit 80 in the refractory block 81 at the side wall of the ladle.

The metal jacket section 46 is provided with an enlarged aperture 82 for receiving the refractory block 83, which may be cylindrical in form, and which is provided with the discharge aperture 23, forming a continuation of the conduit 80.

The refractory block 83 may be housed in a cast metal fitting 84 (Fig. 4), which is provided with an inner curved surface 85, and peripherally extending flanges 86, 87 fit against a metal band 90 surrounding the wall of the section 46, to which the flanges 86, 87 are bolted by means of the screw bolts 88, which have their threaded ends projecting outward from the shell 46.

The fitting 84 may be built up in the form of a plurality of metal sections 90, 91, 92, bolted or otherwise secured together, but the external portion 92 thereof is provided with laterally projecting flanges 93 and vertically projecting flanges 94, forming internally directed guide grooves 95, 96 for receiving a complementary part carried by a mold.

The guide grooves 95, 96 extend parallel to

each other and in straight lines so that the flanges 97, 98 carried by the mold may be slidably mounted in the grooves 95, 96. Each of the molds 100-105 may comprise a metal lining and an external metal jacket 106 formed of two similar halves 107, 108 fitting together.

In other cases the jacket halves 107, 108 are lined with an inner layer 109, 110 of smooth high-temperature-resistant and heat-insulating refractory, previously mentioned, which is used to line the innermost chamber 71 of the ladle, and the refractory sections 109, 110 of the mold have the casting cavity 111 formed in them, and are separable at the same joint 112 as the metal halves 107, 108 of the jacket 106. For the purpose of illustration, the mold 101 is illustrated with a jacket comprising two separable sections which are clamped or bolted together in any suitable way, preferably by means of pivoted bolts 20 and wing nuts so that the molds may be removed quickly at the proper time. However, the molds may be made of any number of sections suitable to the nature of the shape of the casting so as to facilitate the removal of the mold from the casting as soon as it has congealed, without breaking any part of the casting.

The proper number of sections for a jacket or refractory lining of a mold will be evident to any one skilled in the art of molding.

The present molds are adapted to be used over and over again, and are practically indestructible. They are also preheated before use, and are maintained in a heated condition by reuse, the number of molds being adapted to the continuous operation of the machine by the use of a mold practically as soon as it has been removed from one congealed casting which is still at a highly heated condition.

The refractory sections of the mold are formed with the semi-cylindrical grooves 113, 114, which together form an aperture or conduit that increases in size gradually as it extends downwardly and laterally, and the aperture 116 of this conduit 115 fits the discharge aperture 23 of the ladle.

The metal jacket 106 of each mold has a diagonally downward and laterally extending formation which is adapted to be secured to the guide fitting 117, having the flanges 97, 98 previously mentioned. This guide fitting has a pair of outwardly extending flanges 118 and a pair of downwardly and upwardly extending flanges 119, and is provided with set screws 120 for securing to the mold.

It will be noted that in Fig. 4 the mold 101, which is for a relatively flat casting, extends diagonally upwardly. This is for the purpose of permitting the filling of the mold by the flowing upward of the melted metal in the mold, without any splashing or formation of drops.

It is contemplated that no special gates will be required for the discharge of the air in the mold, as the air may leak out between the two halves of the refractory lining and metal jacket of the mold, which are fitted closely enough to mold the casting with practically no fin, but still permit the escape of air.

It will be noted that the reservoir or ladle 20 is formed with a downwardly and laterally extending discharge conduit, which tapers gradually to its smallest section at the mouth 121 of the casting cavity. The molds may thus be slidably supported by means of the guide fixture 84, which is located not only in front of the furnace, but extends longitudinally from the furnace in a

straight line, so as to support a multiplicity of molds, as shown in Fig. 6. In some embodiments of the invention the ladle may be provided with a plurality of discharge openings for an equal number of molds.

In some plants the molds may be shoved past the discharge aperture 23 of the ladle by hand. As soon as the aperture 116 of the mold has passed the discharge aperture 23, the further discharge of melted metal is arrested by the fact that the flat surfaces on the face 122 of the refractory of the mold cover up the discharge aperture 23.

If desired, a suitable steel die may be provided at this face 122 for shearing off any metal which may have congealed.

In the practice of my method, the metal, which may be congealed slightly, will still be capable of being sheared off at this time.

When the molds are shoved into place by hand, there will be suitable stops such as pins, placed in apertures in the fitting 84 for stopping the mold, with the apertures 23 and 116 in registry, and the pulling of the stop pin or movement of the stop member out of its operative position will permit the progress of the mold from the casting position to a position further on in the guides of the guide fixture 84.

In other embodiments of the invention a suitable driving mechanism may be provided, such as, for example, the frame members 130 (Fig. 6) which support a driving rack 131 that is slidably mounted by means of the pins 132 in slots 133 below the molds.

This rock may be spring-urged toward the right by means of a tension spring 134 engaging a pin on the rack, and having its opposite end secured to a frame member. The rack is provided with a plurality of pawls 135-140. Each pawl 135-140 is pivotally mounted upon a pin 141 and engages a stop member 142, toward which it is pulled by means of a spring 143.

The rack bar 131 also has a driving pin 145 suitably located to be engaged by the shoulder 149 carried by a rotating drive wheel 150 mounted on shaft 151.

The operation of this step-by-step mechanism is as follows: Shaft 151 may rotate at a constant speed, which is determined by the length of time required for the making of one casting. This time will be sufficient, as hereinafter more fully described, to permit not only the filling of the mold with melted metal, but the continued application of melted metal under gravity head to the mold while the casting congeals from its outermost point inward toward the supply of metal in the reservoir.

During this congealation the shrinkage of the casting is taken up by the supply of additional metal from the molten end of the casting, and the last part of the casting to freeze should be that adjacent the mouth 121 of the mold. Thus the actuating shoulder 149 performs a rotation in a predetermined time, which is determined by the characteristics of the casting or mold and by the time required to carry out my process.

When the shoulder 149 engages the pin 145, it causes the rack 131 to move to the left by an amount equal to the length of a slot 133, which is sufficient to move one mold 101 from the position which it occupies in Fig. 5, in registry with the discharge aperture 23, and to bring the next mold 102 into that same position. Thereafter the shoulder 149 slips off and passes the pin 145, due to the rotation of the wheel 150, and the

spring 134 returns the rack 131, during which movement all of the pawls 135-140 are adapted to slide past the molds which are immediately to the right of each pawl.

5 The pawls are then in position to engage and actuate these molds when the rack has reached the position of Fig. 6 again. Thus the mechanism is adapted to effect the movement of the molds in a step-by-step manner and to permit 10 the molds to remain in casting position for a predetermined length of time.

Referring again to Fig. 4, the ladle is preferably provided with a fixed cover member 160, which may comprise a metal jacket 161 having an 15 external cylindrical portion 162 and a flat end portion 163.

The jacket 161 may be bolted in place by means of the bolts 164 and flanges 165, 166. The jacket may have a centrally located aperture 167 with a 20 downwardly extending frusto-conical flange 168. The jacket is lined with a flat block of refractory 169 in the form of a disc having a centrally located frusto-conical bore 170 fitting against the flange 168.

25 This aperture 170 serves as a filling opening for the reservoir or ladle 71, and it in turn may be closed by a movable cover member 171, which has a metal jacket 172 and a refractory lining 173 retained by means of a frusto-conical flange 174. The movable cover 171 fits in the bore 167 and produces an effective closure, due to the engagement of the metal flanges 168 and 174.

30 The movable cover 171 may be provided with a centrally located air aperture 175, communicating with a counterbore 176 for receiving a conical valve member 177. The valve member 177 has a stem 178 guided in an aperture in the jacket 172 and urged to closed position by a 35 spring 179. The stem 178 has a transverse pin 180 engaging in a slot in the end of a lever 181.

35 The lever 181 is pivoted on the bracket 182 and provided at its opposite end with a pull rod 183 slidably mounted in a guide fixture 184 and provided with a ball counter-balance 185. By means 40 of a pull on the rod 183 the operator may regulate the admission of air to the chamber 71 of ladle 20, and thus control, at least in some measure, the discharge of metal from its lower end.

45 Thus the pull rod 183 would be pulled whenever the mold was in front of the discharge aperture of the ladle, and the actuation of the rod may be gradual, in order to permit the filling of the mold without any splashing, or to reduce the impact which results when the molten metal flowing into the mold reaches the end of the mold.

50 Referring to Fig. 5, this is a modification in which the conduit 115 is provided with a butterfly valve 270 for controlling the flow of the metal into the mold.

55 This valve may be so constructed that its actuating shaft may be withdrawn, and that portion of the conduit 115 surrounding it may be separated when the mold is separated, so that the metal in the conduit 115 may be removed from the conduit with the valve 270, and a new valve substituted when the mold is again used.

60 My method of casting is briefly described as follows: When a ladle of the type described is used, the ladle is constantly supplied with new batches of molten metal, from which all dross or scum have been removed in the furnace, and this metal is supplied to the ladle without exposure to the air, so far as possible.

65 A de-oxidizer compound may be kept on top of the charge, to prevent air contamination.

The molten metal is kept in the ladle, which is lined with smooth refractory, suitably treated with flux or charcoal, to prevent the metal from sticking to it, and suitably insulated, so that the metal may be maintained at a high temperature, with a minimum fluctuation of temperature between batches.

When ordinary castings are to be made, the mold is made of a similar smooth refractory capable of retaining the heat, and providing heat insulation for the casting, and the mold is pre-heated either by a preheating operation or by being used over and over again, immediately after a previous casting operation.

The mold and the ladle have their entry and discharge openings and conduit for the metal smoothly tapered along stream lines so that there will be no splashing and the least amount of agitation of the metal.

The mold may be lined with metal inside the refractory to reduce breakage of molds and improve castings and when casting with certain metals, I use metal molds where it is economical.

The mold is tilted upward from its filling opening so that metal running into the mold cannot drop down to the end of the mold and splash. After the mold opening is placed in registry with the discharge opening of the ladle, the molten metal is permitted to well up into the mold, its level constantly rising, until it completely fills the mold.

During this time the metal is still molten and maintained heated because of the insulating character of the refractory mold or the pre-heating of the mold.

The mold may, in the case of relatively large castings, be provided with apertures for the issuance of the air, but in most cases the air will leak out between the halves of the mold, and the molds in such case will not need risers.

The method may be practised with all types of metals. The thickness of the refractory in the mold and in the ladle are proportionate to the bulk of the metal in the casting or the bulk of the metal in the ladle, respectively.

After the mold has been filled, it is then maintained in the same position, with the metal of the ladle pressing into the mold, due to the head of the metal in the ladle, until the metal has solidified in the mold.

During this operation the pouring end of the mold is the hottest, and the end farthest from the ladle is the coolest. There is a heat gradient extending from the ladle outward to the extreme end of the mold. As the metal solidifies, it begins to solidify at the extreme end of the mold, away from the ladle, and gradually solidifies downward toward the filling opening of the mold. During this operation any shrinkage is taken up by the supply of additional melted metal, due to the head of the metal in the ladle.

There will be no flaws or pipes, nor will the casting be subjected to strains due to unequal contraction. The entire mold will be filled, and the casting will correspond more closely to the shape of the mold than with the methods of the prior art.

After the casting has solidified in the mold down to the filling opening of the mold, the further flow of metal into the mold is cut off by sliding the mold sidewise so that the stream of metal is sheared off. If it has solidified down to the point of shearing, it can still be sheared off, due to its relative softness at such a high

temperature, and the discharge aperture of the ladle is closed by a flat surface on the end of the mold.

The next mold continues to close this discharge opening by a similar flat surface until its filling opening comes in registry with the discharge opening of the ladle, after which the filling of mold is again resumed.

10 The mold, which has been filled and removed from its ladle, has its parts separated, and the casting is removed at a proper time, which is determined by the character of the casting. This enables the use of the mold over again while it is still in a heated condition, and the casting may contract as it cools, without producing any strains on the mold or breaking the mold. The casting may contract more freely than if it were left in the mold.

15 Castings may thus be made to closer tolerances, and the present method makes sure the elimination of flaws because of the constant application of liquid metal under pressure to the molten side of the casting, as the casting solidifies. There is no chance of getting drops of metal in the mold, as the metal wells up into the mold, due to the tilt of the mold with respect to its filling opening.

20 Such drops frequently happen in the casting methods of the prior art on account of splashing or agitation, and such drops solidify on the way down into the mold, in the devices of the prior art. This cannot happen according to my method.

25 One of the most important features of the method is the freezing of the metal last at the mouth of the mold and at the beginning of the freezing at the point farthest away from the mouth of the mold. In some castings gates may be provided at the most remote point of the mold. A rim around the casting may usually be avoided because such heavy pressures are not employed in my method as in die casting.

30 The castings, after removal from the mold, are preferably subjected to the uniform foundry temperature of approximately 65 degrees F., and kept out of draft. They could also be quenched in water, if desired, but are preferably cooled uniformly by being subjected to a moderate and uniform cooling temperature so that they will contract in proportion, everywhere in the casting.

35 While I have illustrated a preferred embodiment of my invention, many modifications may be made without departing from the spirit of the invention, and I do not wish to be limited to the precise details of construction set forth, but desire to avail myself of all changes within the scope of the appended claims.

40 Having thus described my invention, what I claim as new and desire to secure by Letters Patent of the United States, is:

45 1. The method of casting which comprises melting the casting metal in a plurality of melting furnaces arranged to provide batches of molten metal for discharge into a ladle at regular intervals to maintain the head of metal in said ladle at predetermined height and to maintain the high temperature of metal in said ladle, maintaining the temperature of the metal in said ladle by insulation and by periodic supply of hotter metal, discharging the molten metal from said ladle at its lower end laterally and upwardly into a mold having a cavity and a downwardly directed filling opening, the molten metal welling up into said mold to fill the mold without splash-

ing, and with a minimum contact of molten metal to the air in the mold, maintaining the temperature of the casting metal in the mold cavity by insulation of said mold, and keeping the mold in connection with the supply of molten metal while the metal solidifies in the mold, beginning at a point remote from the filling opening, downward to the filling opening, whereby the shrinkage is taken up by the supply of additional molten metal from said ladle until the casting is solidified to its filling opening, successively applying similar molds to said discharge opening of said ladle, and removing the molds from the castings after filling and congelation, to permit the free contraction of the casting without interference of the mold while cooling.

2. The method of casting which comprises providing a supply of molten metal in an insulated container, and maintaining the temperature of said metal at a predetermined temperature, transferring molten metal at said predetermined temperature from said container directly into a mold, through a relatively large stream-lined discharge opening, the transfer of metal from ladle to mold being from a point below the free surface of the molten metal in the container at the time of transfer, and said mold having its cavity extending upward from said discharge opening at the time of transfer, the transfer of the metal from container to mold taking place in the form of a gradual welling up of a solid stream of metal in the mold without splashing or spouting or separation of molten metal from the main body of said stream until the mold is filled by gravity head, and thereafter maintaining a gravity head pressure on said mold in excess of the head of metal in said mold for a predetermined period of time to supply metal to the interior of the casting during congelation and shrinkage, the casting solidifying from a point farthest from said discharge opening down toward said discharge opening.

3. The method of casting which comprises providing a supply of molten metal in an insulated container, and maintaining the temperature of said metal at a predetermined temperature, transferring molten metal at said predetermined temperature from said container directly into a mold, through a relatively large streamlined discharge opening, the transfer of metal from ladle to mold being from a point below the free surface of the molten metal in the container at the time of transfer, and said mold having its cavity extending upward from said discharge opening at the time of transfer, the transfer of the metal from container to mold taking place in the form of a gradual welling up of a solid stream of metal in the mold without splashing or spouting or separation of molten metal from the main body of said stream until the mold is filled by gravity head, and thereafter maintaining a gravity head pressure on said mold in excess of the head of metal in said mold for a predetermined period of time to supply metal to the interior of the casting during congelation and shrinkage, the casting solidifying from a point farthest from said discharge opening down toward said discharge opening, and removing said casting from its mold promptly after solidification of the metal of the casting down to said discharge opening.

4. The method of making metal castings of homogeneous uniform-grained structure which comprises melting a supply of clean metal in a plurality of furnaces arranged adjacent a heat

insulated ladle, to a predetermined elevated temperature, maintaining a supply of said melted metal in the heat insulated ladle at a predetermined lower temperature by periodically discharging metal successively from said furnaces into said ladle, discharging the molten metal from said ladle at a point below the free surface of the metal directly into a preheated metal mold constructed of a metal of higher melting point than the casting metal, said mold extending upward from its filling opening, whereby the metal wells upward into the mold without splashing due to the gravity head of metal in the ladle until the mold is filled, maintaining the gravity head on the metal in the mold thereafter in excess of the head of metal in said mold for a predetermined period of time to supply metal to the interior of the casting during congelation and shrinkage, the casting cooling naturally by radiation and conduction and solidifying from a point farthest from said discharge opening and inwardly from the sides of said mold down toward the discharge opening and stopping the application of pressure head to said casting when the casting has congealed just past the filling opening of the mold.

5. The method of making metal castings of homogeneous uniform-grained structure which comprises melting a supply of clean metal in a plurality of furnaces arranged adjacent a heat insulated ladle, to a predetermined elevated temperature, maintaining a supply of said melted metal in the heat insulated ladle at a predetermined lower temperature by periodically discharging metal successively from said furnaces into said ladle, discharging the molten metal from said ladle at a point below the free surface of the metal directly into a preheated metal mold constructed of a metal of higher melting point than the casting metal, said mold extending upward from its filled opening, whereby the metal wells upward into the mold without splashing due to the gravity head of metal in the ladle until the mold is filled, maintaining the gravity head on the metal in the mold thereafter in excess of the head of metal in said mold for a predetermined period of time to supply metal to the interior of the casting during congelation and shrinkage, the casting cooling naturally by radiation and conduction and solidifying from a point farthest from said discharge opening and inwardly from the sides of said mold down toward the discharge opening and stopping the application of pressure head to said casting when the casting has congealed just past the filling opening of the mold, the said ladle and mold being closed to minimize the oxidation of metal at the free surface, and the mold being heat insulated to eliminate the possibility of cooling by extraneous influences.

6. The method of making metal castings of homogeneous uniform-grained structure which comprises melting a supply of clean metal in a plurality of furnaces arranged adjacent a heat insulated ladle, to a predetermined elevated temperature, maintaining a supply of said melted metal in the heat insulated ladle at a predetermined lower temperature by periodically discharging metal successively from said furnaces into said ladle, discharging the molten metal from said ladle at a point below the free surface of the metal directly into a preheated metal mold constructed of a metal of higher melting point than the casting metal, said mold extending upward from its filling opening, whereby the metal

wells upward into the mold without splashing due to the gravity head of metal in the ladle until the mold is filled, maintaining the gravity head on the metal in the mold thereafter in excess of the head of metal in said mold for a predetermined period of time to supply metal to the interior of the casting during congealation and shrinkage, the casting cooling naturally by radiation and conduction and solidifying from a point farthermost from said discharge opening and inwardly from the sides of said mold down toward the discharge opening and stopping the application of pressure head to said casting when the casting has congealed just past the filling opening of the mold, and separating the casting and mold promptly after solidification to permit the shrinkage of the casting without constraint.

7. The method of making metal castings of homogeneous uniform-grained structure which comprises melting a supply of clean metal in a plurality of furnaces arranged adjacent a heat insulated ladle, to a predetermined elevated temperature, maintaining a supply of said melted metal in the heat insulated ladle at a predetermined lower temperature by periodically discharging metal successively from said furnaces into said ladle, discharging the molten metal from said ladle at a point below the free surface of the metal directly into a preheated metal mold constructed of a metal of higher melting point than the casting metal, said mold extending upward from its filling opening, whereby the metal wells upward into the mold without splashing due to the gravity head of metal in the ladle until the mold is filled, maintaining the gravity head on the metal in the mold thereafter in excess of the head of metal in said mold for a predetermined period of time to supply metal to the interior of the casting during congealation and shrinkage, the casting cooling naturally by radiation and conduction and solidifying from a point farthermost from said discharge opening and inwardly from the sides of said mold down toward the discharge opening and stopping the application of pressure head to said casting when the casting has congealed just past the filling opening of the mold, the stopping of said pressure head to said casting being accomplished by lateral movement of the mold with respect to the discharge opening of the ladle, bringing the mold and ladle out of registry, and successively moving a plurality of similar molds into and out of registry with the discharge opening of said ladle at a predetermined periodic rate to make a plurality of castings of uniform characteristics. 55

8. The method of making metal castings having a homogeneous uniform-grained structure, which comprises providing a supply of clean molten metal in a heat insulated container, discharging the molten metal from said container at a point below the free surface of the molten

metal directly into a preheated mold constructed of material of higher melting point than the casting metal, said mold having its major axis extending upward from its filling opening at an angle which is oblique with respect to the free surface of the molten metal, whereby the metal wells upward into the mold in a solid stream of metal without splashing or spouting or separation of molten metal from the main body of said stream, with its free surface progressing upward from the filling opening to the top of the mold, until the mold is filled by gravity head, and thereafter maintaining a gravity head pressure on the metal in said mold by means of the molten metal in said container, in excess of the head of the metal in said mold for a predetermined period of time to supply metal to the interior of the casting during congealation and shrinkage, the casting cooling and solidifying from a point farthest from said discharge opening, and inwardly from the sides of said mold down toward the discharge opening, and causing the cessation of the application of pressure to said casting when the casting has congealed to a predetermined point.

23 9. The method of making metal castings having  
1 a homogeneous uniform-grained structure, which comprises providing a supply of clean  
1 molten metal in a heat insulated container, dis-  
30 charging the molten metal from said container  
at a point below the free surface of the molten  
metal directly into a preheated mold constructed  
of material of higher melting point than the  
35 casting metal, said mold having its major axis  
extending upward from its filling opening at an  
angle which is oblique with respect to the free  
surface of the molten metal, whereby the metal  
wells upward into the mold in a solid stream of  
40 metal without splashing or spouting or separa-  
tion of molten metal from the main body of said  
stream, with its free surface progressing upward  
from the filling opening to the top of the mold,  
until the mold is filled by gravity head, and  
45 thereafter maintaining a gravity head pressure  
on the metal in said mold by means of the molten  
metal in said container, in excess of the head of  
the metal in said mold for a predetermined  
period of time to supply metal to the interior of  
50 the casting during congealation and shrinkage,  
the casting cooling and solidifying from a point  
farthermost from said discharge opening, and  
inwardly from the sides of said mold down to-  
ward the discharge opening, and causing the ces-  
55 sation of the application of pressure to said cast-  
ing when the casting has congealed to a prede-  
termined point, and removing said casting from  
its mold promptly after solidification of the metal  
of the casting to permit the casting to contract  
without the restraint of the mold.

CARL WESSEL